

## UNITED STATES PATENT OFFICE.

LAWRENCE E. BARRINGER, OF SCHENECTADY, NEW YORK, ASSIGNOR TO GENERAL ELECTRIC COMPANY, A CORPORATION OF NEW YORK.

## MOLDED MATERIAL AND METHOD OF PREPARATION.

No Drawing.

Application filed March 31, 1922. Serial No. 548,535.

*To all whom it may concern:*

Be it known that I, LAWRENCE E. BARRINGER, a citizen of the United States, residing at Schenectady, county of Schenectady, State of New York, have invented certain new and useful Improvements in Molded Materials and Methods of Preparation, of which the following is a specification.

10 The present invention comprises improved molded materials which contain as a constituent fibrous material, as for example, asbestos, wood fibre or textile fibres, such as cotton. My invention, which also includes 15 a new process, is particularly applicable to the manufacture of electrical insulators.

It is the object of my invention to improve products of this class both by the more uniform and thorough distribution of 20 a binder, and also a more complete purification of the material than was heretofore practicable.

In accordance with my invention fibrous materials when cleaned from conducting 25 particles are converted to sheet form,—that is to a paper or cloth. The sheet material is coated with a suitable binder, which hardens at room temperature but is capable of being softened by heat. The coated product 30 is shredded and finally compacted by pressure to desired form.

My invention is particularly applicable to the manufacture of molded asbestos products. There is a considerable amount of 35 undesirable matter in native asbestos mineral, particularly iron oxide, which is a fairly good conductor and is removable only with the greatest difficulty. When the asbestos is converted to a pulp and admixed with 40 acids for chemical purification, a flocculent fibre is produced which is mixed with a binder with difficulty. By coating the material in sheet form the most complete and uniform distribution of the binder is secured 45 and less binder required for a given quantity of fibrous material.

In carrying out my invention, asbestos, and other fibrous materials, are suitably cleansed, then converted into paper form 50 and coated with shellac or natural or synthetic resins as bakelite, or with varnish,

or other suitable binding material which normally becomes hard at room temperature, but possess plasticity at high temperature. In general, binders of this class may 55 be called thermoplastic materials.

The coated paper or fabric, is shredded mechanically by suitable mechanism, such, for example, as machines containing revolving knives and known to the trade as rotary 60 cutters or shredding machines. The subdivided material finally is compressed in molds with or without admixture of fillers, or additional binders. To obtain the proper results the mold should be heated to the 65 softening temperature of the binder.

Various other materials now used in molded compositions in an impure condition and not easily mixed with binders because of their physical condition, to advantage, 70 may be converted to sheet form and then coated and shredded in accordance with my invention. Wood fibre and cotton flock are examples. These materials can readily be purified chemically before conversion to a 75 paper or cloth.

Waste material resulting from factory processes utilizing coated fabric may be utilized to advantage in accordance with my invention by shredding the same and mold- 80 ing the product as above described.

What I claim as new and desire to secure by Letters Patent of the United States, is,—

1. A molded material comprising a heat compacted mass of shredded sheet material 85 having a coating of thermoplastic binder.

2. The method of making molded material which consists in coating fibrous material in sheet form with a thermoplastic material, then subdividing said sheet material 90 and finally molding the product under heat and pressure.

3. The method of making molded asbestos products which consists in coating sheet asbestos with a binder which softens at ele- 95 vated temperature, shredding the coated product and molding the shredded material under pressure at the softening temperature of said binder.

In witness whereof, I have hereunto set 100 my hand this 30th day of March, 1922.

LAWRENCE E. BARRINGER.